

April 5, 1927.

1,623,555

J. G. ROBERTS

LOADED SIGNALING CONDUCTOR

Filed Aug. 16, 1921



Inventor:  
John G. Roberts,  
by *Jed C. Palmer* Atty.

## UNITED STATES PATENT OFFICE.

JOHN G. ROBERTS, OF DOBBS FERRY, NEW YORK, ASSIGNOR TO WESTERN ELECTRIC COMPANY, INCORPORATED, OF NEW YORK, N. Y., A CORPORATION OF NEW JERSEY.

## LOADED SIGNALING CONDUCTOR.

Application filed August 16, 1921. Serial No. 492,743.

This invention relates to loaded signaling conductors and particularly to continuously loaded conductors suitable for submarine cables.

5 An object of the invention is to provide a stranded signaling conductor on which the loading material is so positioned that it will suffer no displacement when the cable in which the conductor is incorporated is 10 submerged.

Another object is to provide a loaded signaling conductor of high efficiency and one whose efficiency does not vary materially.

The drawing shows a cross-section of the 15 cable made in accordance with this invention.

The signaling conductor consists of a central wire 1 surrounded by six wires 2. The conductor is preferably formed by stranding 20 the outer wires around the central wire 1. Such a conductor has proven to be desirable in order that the cable may be as flexible as possible and thus reduce any tendency to become disrupted either during the 25 process of laying or while in actual use. Instead of employing a conductor like that shown in the drawing, it may be desirable for particular purposes to employ other well known types of cable conductors, such, for example, 30 as a structure in which no central core is employed or one employing a core of insulating material.

In applying continuous loading to this 35 sort of a conductor when iron is used as the loading material, the tape or wire is wrapped thereabouts, touching the composite conductor at relatively few points. Upon the submergence of the cable, the excessive water pressure forces the loading material 40 into the interstices between the outer wires, causing strains and stresses to be set up in the magnetic material. Such strains and stresses do not materially affect the permeability of the iron, and for this reason 45 the change in position of the tape or wire is not of any great moment.

It has been found, however, that when 50 material of high permeability at low magnetizing forces is employed, such as for example, certain alloys of nickel and iron, this change of position seriously impairs its magnetic properties due to the excessive strains and stresses set up therein. This invention provides a method of so positioning the load-

ing material about the conductor that no 55 change in position thereof relative to the conductor, results from the submergence of the cable, thus preventing any impairment in the permeability of the magnetic material.

In accordance with the invention, the magnetic tape or wire 3 is initially compressed 60 about the conductor, so that its inner surface is substantially at all points in contact with the conductor. This may be accomplished in a variety of ways, the preferred method being to draw the conductor after the loading material has been applied, through a suitable die which will force the tape or wire into the interstices between the outer wires. When 65 this is done the contour of the magnetic material conforms to the contour of the conductor. The loading wire or tape is preferably well annealed before wrapping so that it will conform readily to its new position when passed through the die.

To develop the utmost permeability in the magnetic material the loaded conductor may be subjected to a heat treatment, the treatment required in any particular case varying 70 somewhat as regards temperatures employed and duration of heating and cooling. The optimum values of these variables may be readily determined in any specific case by experiment. After the heat treatment, the material should be guarded against any considerable strains.

75 After the heat treatment, insulating material 4, such as gutta percha, is applied to the loaded conductor in accordance with the usual method of insulating submarine conductors. Loading materials as referred to hereinbefore are described in the patent to Elmen No. 1,586,884, granted June 1, 1926.

80 What is claimed is:

1. A signaling conductor having an uneven surface, and a layer of magnetic material wrapped spirally about the conductor and pressed into intimate mechanical contact therewith to conform to the surface of the conductor.

85 2. The method of loading a signaling conductor having a plurality of cylindrical wires, which comprises wrapping the conductor helically with magnetic material and forcing said material into intimate contact 90 with substantially the entire exterior surface of said conductor.

95 3. The method of loading a signaling con-

ductor having a plurality of cylindrical wires, which comprises helically wrapping the conductor with a layer of loading material and shaping the loading material to conform to the contour of said conductor.

4. The method of applying a magnetic sheath to a stranded conductor, which comprises wrapping said conductor with a helical covering of magnetic tape, and compressing said magnetic tape into the crevices between the strands of the conductor so that

the magnetic sheath conforms to the contour of the conductor.

5. A signaling conductor comprising a plurality of wires stranded together and having a continuous strip of magnetic material wrapped helically about said conductor and compressed into the interstices thereof.

In witness whereof, I hereunto subscribe my name this 10th day of August, A. D., 1921.

JOHN G. ROBERTS.